

1

2,776,749

## ALKOXY BENZENE IN FROTH FLOTATION PROCESS

Roger F. Powell, Gwelo, Southern Rhodesia, and Eric F. Martin, Germiston, Transvaal, Union of South Africa, assignors, by direct and mesne assignments, to National Chemical Products Limited, Germiston, Transvaal, Union of South Africa

No Drawing. Application August 2, 1954,  
Serial No. 447,441

Claims priority, application Great Britain June 14, 1949

8 Claims. (Cl. 209—166)

The present application is a continuation-in-part of our co-pending application Serial No. 167,912, filed June 13, 1950, which has since matured as U. S. Pat. No. 2,687,214, granted Aug. 24, 1954.

The present invention is directed to a method of concentrating minerals by flotation comprising adding a small quantity of an alkoxy substituted benzene compound to the mineral pulp, said alkoxy benzene compound acting as a frother and improving the resulting flotation operation in the separation of the minerals from the impurities associated therewith.

The froth flotation processes of the present invention are particularly suitable for the concentration of noble and base metal ores and provide for a wide range of frothers for selection under the best conditions for the treatment of widely varying mineral compositions.

The froth flotation agents of the present invention are particularly adapted for the treatment of pyritic ores or cyanide slime plant residues of the type where recovery by flotation has presented great difficulties using the methods hereto available. The present frothers are likewise suitable for use with ores containing tarnished pyrite, chalcocite, and ores of the complex lead-zinc type.

The flotation process of the present invention may be used with good advantage in the treatment of gold ores containing small amounts of sulfides or arsenides, the bulk treatment of copper ores containing siliceous gangue and the treatment of ores in which two or more base metals are to be separated from each other, such as copper, lead, zinc or the like. The process may likewise be used for the separation of coal, for instance, of the coking and non-coking type.

The alkoxy benzene compounds of the present invention include benzenes substituted with at least one and up to four alkoxy substituents, the benzene ring being connected to the alkoxy substituent by an ether C—O—C linkage, alkoxy being selected from the group consisting of methoxy, ethoxy, normal propoxy, isopropoxy, methoxy-ethoxy and ethoxy-ethoxy. It is preferred to use alkoxy benzene froth flotation agents which are substituted with at least two of such alkoxy groups. The alkoxy benzenes includes the dialkoxy benzenes, tri-alkoxy benzenes and tetraalkoxy benzenes. The tetraalkoxy benzene may be 1,2,3,5 tetramethoxy benzene. The trimethoxy benzene may be 1,2,3 trimethoxy benzene or 1,3,5 trimethoxy benzene or 1,2,3 trimethoxy benzene. The dimethoxy benzenes may be the ortho, meta or para isomers.

Generally, all of the isomers of the di, tri and tetra alkoxy benzenes, alkoxy as above defined, are each equally suitable within any particular substitution class and as will be evident from the more detailed description set forth below.

The dialkoxy benzenes are prepared by conventional procedures and are also available commercially. The

2

trialkoxy benzenes are prepared in conventional manner by the alkylation of the corresponding trihydric phenols such as phloroglucinol, pyrogallol, etc. The tetraalkoxy benzenes may be prepared through oxidation of the corresponding trialkoxy compounds whereby benzoquinones are formed, the benzoquinones are then reduced to the benzohydroquinone and the latter alkylated to add on the two alkoxy groups to the hydroquinone derivative and produce the desired product. For example, 1,2,3,5 tetramethoxy benzene is obtained by oxidizing pyrogallol trimethyl ether to 2,6 dimethoxy benzoquinone, the latter reduced to 2,6 dimethoxy benzohydroquinone whereafter methylation with dimethyl sulfate in 20% aqueous NaOH and in the absence of air produces the desired 1,2,3,5 tetramethoxy benzene. The other alkoxy derivatives may be prepared in like manner, the alkylating agent being modified as is well known in order to introduce the desired alkoxy substituents.

It is convenient to summarize the essential properties of frothers of interest in froth flotation processes, when used in conjunction with any of the commonly known promotor and/or conditioners, as follows:

- i. That a small quantity of the frother per unit quantity of the ore or other material treated shall suffice to obtain the desired effect.
- ii. Rate of dispersability of the frother in an aqueous ore or like pulp to which it is added.
- iii. "Carrying or collecting power"—a term already understood in the art.
- iv. Selectivity of the frother in its action upon the different minerals or other substances in association with one another in the pulp or the like, each of which having to be floated and, as far as possible, floated separately.
- v. Selectivity of the frother in its action as between minerals or other materials which it is desired to float, and gangue or the like which it is desired not to float.
- vi. Persistence of the frother in recirculation.

Adverting to the feature that organic compounds embraced within the range herein set forth and utilizable individually as effective frothing agents, are readily miscible with one another with the important result that means are thereby afforded in flotation practice enabling the frother by selective mixture to be varied in such a way as to combine in desired proportion essential properties each possessed by the individual substances in different degrees to suit special characterization of a given ore, coal or other material to be treated, this aspect of the present invention will now be more fully discussed.

From a knowledge of the particular flotation properties of individual species in the range of compounds herein set forth, blends of any two or more of these substances can be produced with predictable flotation properties.

Advantages accruing from the foregoing are very substantial, as will appear from the following:

1. Large quantities of cheap species can be blended with smaller quantities of expensive species for economic reasons;
2. Species, one or other of whose properties exclude or substantially exclude them from the range of practical effectiveness when used alone, can be combined to bring such properties within the useful range by intelligent blending of such species with one another.

Adverting to the discussion of the principal practical properties of any frother as appearing earlier herein—

- i. *Selectivity as between two or more valuable minerals which are required to be floated as far as possible separately.*—This property of selectivity is substantially inversely proportional to "collecting-power," a fact which opens up wide possibilities in the result of blending suitably selected compounds.

ii. *Deleterious tendency to float valueless gangue with valuable minerals.*—It has already been established that this tendency is possessed by those species in which the alkoxy group is isopropoxy. Also there is little, if any, increase in this deleterious property as one increased the number of any specific alkoxy groups in the molecule.

For the flotation treatment of particular ores and the like, specific frothers may thus be produced by blending suitable members of the series having regard to the foregoing. As is well known, three main types of ore are met with, namely—

(a) Gold ores in which a comparatively small percentage of sulfides or arsenides individually rich in gold require to be concentrated by flotation, in which case the desideratum is maximum recovery of these auriferous minerals, while the floating of a little extra gangue can be tolerated.

(b) Bulk flotation of one or more minerals of one base metal, e. g. copper, in which case while maximum economic recovery is naturally highly desirable it is absolutely essential that the minimum of siliceous gangue shall be present in the final concentrate.

TABLE I.—STANDARDISED "PRELIMINARY WATER-FROTHING TEST" ON A NUMBER OF POTENTIAL FROTHERS

[Long experience has shown that this test gives a very fair indication of the comparative behavior of potential frothers, roughly quantitatively. "Net commercial strength" and qualitative properties have to be determined on actual ores.]

|               | Formula of Compound | Physical State                   | Approximate Quantity needed to start good froths (without viscosity correction) | Approximate Quantity needed for froth to "Run Over" |
|---------------|---------------------|----------------------------------|---------------------------------------------------------------------------------|-----------------------------------------------------|
| 1.            |                     | Liquid-----                      | 0.09 cc-----                                                                    | 0.24 cc.                                            |
| 2.            |                     | Liquid-----                      | 0.22 cc-----                                                                    | 0.36 cc.                                            |
| 3.            |                     | Solid; used 10% w.v. in alcohol. | 0.26 g-----                                                                     | 0.41 cc.                                            |
| 4.            |                     | Solid; used 5% w.v. in alcohol.  | 0.05 g-----                                                                     | 0.07 g.                                             |
| 5.            |                     | Solid; used 50% w.v. in alcohol. | 0.045 g-----                                                                    | 0.105 g.                                            |
| PINE OIL----- |                     | Liquid-----                      | 0.057 cc-----                                                                   | 0.114 cc.                                           |
|               |                     | Liquid-----                      | 0.015 cc-----                                                                   | 0.030 cc.                                           |
|               |                     | Liquid-----                      | 0.045 cc-----                                                                   | 0.075 cc.                                           |

<sup>1</sup> All soluble with great ease in pure 1:1:3-triethoxybutane or Commercial 1:1:3 Triethoxybutane.

(c) Ores in which minerals of two or more base metals are to be separated as far as possible from each other as well as from the gangue; in which case the desiderata are extreme selectivity coupled with deep and powerful froth while at the same time maximum "carrying-power" is desired in the second or final stage of flotation.

As regards coal separation the first desideratum is extreme selectivity to permit the separation of two or more basic types of coal, as for instance, "coking" and "non-coking" coal.

An object of the invention is to provide improved froth flotation agents for the flotation of mineral pulp which alone or in various combinations with members of the specified class, polyalkoxy benzenes, alkoxy defined as selected from the group consisting of methoxy, ethoxy, normal propoxy, isopropoxy, methoxy-ethoxy and ethoxy-ethoxy provide improved selectivity and improved flotation results to satisfy the requirements indicated hereinabove.

A further object of the invention is to provide a method for concentrating minerals by flotation comprising adding to the mineral pulp a small quantity of a polyalkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

Other and further objects of the present invention will appear from the more detailed description set forth below, it being understood that such detailed description is given by way of illustration and explanation only and not by way of limitation, since various changes therein may be made by those skilled in the art without departing from the scope and spirit of the present invention.

#### EXAMPLE 1

##### Standard water frothing test

A 5% solution of the following polyalkoxy benzenes are prepared in ethyl alcohol (absolute) and these 5% solutions were added in the amounts specified in Table I below in order to determine the amount necessary to start a good froth and the amount necessary to make the froth run over, these amounts being placed on the same frothing basis as pine oil, a well known standard frother.

The standard "water-frothing test" (see the penultimate item of Table I of specification) shows that 0.015 gram suffices to start good froths, and 0.025 gram were needed to make the froths "run over." Triethoxybenzene is a great deal stronger than the trimethoxybenzene, just as it can be seen that the para-diethoxybenzene is a great deal stronger than the para-dimethoxybenzene.

The test was made with a 5% solution of the 1,2,3 triethoxybenzene in absolute ethyl alcohol, which solvent is known to have no further power in such quantities as were used.

It is noted that 1,2,3 triethoxybenzene has a melting point of 39° C., so is a solid at usual room temperatures. Its solubility in water is so low that even in warm water it was found impossible to prepare a 0.5% solution. This is in contrast to the 1,2,3 trimethoxybenzene, which for certain flotation tests is used as a 0.5% aqueous solution.

It is soluble completely and with great ease in commercial triethoxybutane frother.

It is very soluble in absolute ethyl alcohol.

#### EXAMPLE 2

##### Pyritic ore

The material treated is a "cyanide slime plant residue": the flotation problem is to concentrate as much pyrites as possible, as quickly as possible, in a concentrate of as high a grade as possible, with the lowest possible con-

sumption of frothing agent. Pulp density was approximately 36% solids; the machine used a 2000-gram Fahrenwald; conditioning agents H<sub>2</sub>SO<sub>4</sub> to give a pH of 5.3, CuSO<sub>4</sub> as a cyanide; promoting agent 0.10 lb. per ton of sec. butyl xanthate; and frothing agent a 5% solution of the 1,2,3 triethoxybenzene in absolute ethyl alcohol.

The addition of 0.015 lb. triethoxybenzene per dry ton of ore gave a concentrate, 10.59% by weight, assaying 36.11% sulphur, and containing 91.9% of the pyrites originally present in the ore. Period of flotation 3 minutes.

Addition of a further 0.015 lb./ton gave a middling, 2.06% by weight, assaying 7.62% sulphur, and containing a further 3.8% of the pyrites originally present in the ore. Period of flotation a further 5 minutes.

The tailings, 87.35% by weight, assayed 0.204% sulphur, and contained 4.3% of the pyrites originally present in the ore.

The froths were desirably active and rather brittle.

#### EXAMPLE 3

##### Control test with commercial 1,1,3 triethoxybutane

The run was made as in Example 2 above.

The corresponding figures were: Addition of 0.060 lb. of triethoxybutane/ton gave a concentrate 14.54% by weight, assaying 28.42% sulphur, and containing 93.0% of the original pyrites. Flotation time is 3 minutes. Then, without further addition of frother, the middling, 2.31% by weight, assayed 4.04% sulphur, and contained a further 2.1% of the pyrites. Flotation time, a further 5 minutes. The tailings, 83.15% by weight, assayed 0.261% sulphur, and contained 4.9% of the original pyrites.

#### EXAMPLE 4

##### Comparison with Dow froth 250

1,2,3 trimethoxybenzene is compared with Dow froth 250, one of the best flotation agents available at the present time for the flotation of lead-zinc ore. In this type of ore it is desirable to produce a brittle froth and it is important that the action be fast and selective.

1,2,3 trimethoxybenzene is identified as No. 4 frother below.

No. 4 frother is a solid consisting of slightly amber colored crystals, soluble in hot water. A 0.5% solution is made up and used for the flotation tests. In this form its action is fast and it forms a fine brittle froth of good depth, and is maintained to the end of the float. On one or two floats the froth produced was too brittle and the froth bed was shallower than normal. Flotation results are good.

Comparative flotation tests were made using standard test procedure. Floats were made at a pulp temperature of 20° C.

##### No. 4 FROTHER USED, AVE. OF 6 TESTS

|          | Percent Wt. | Percent Assays |      |      | Percent Distribution |       |       |
|----------|-------------|----------------|------|------|----------------------|-------|-------|
|          |             | Pb             | Zn   | Fe   | Pb                   | Zn    | Fe    |
| Pb Conc. | 8.7         | 41.0           | 13.8 | 15.8 | 82.4                 | 22.5  | 6.8   |
| Zn Conc. | 8.8         | 4.3            | 41.6 | 15.4 | 8.8                  | 68.7  | 6.8   |
| Tails    | 82.5        | 0.46           | 0.57 | 21.0 | 8.8                  | 8.8   | 86.4  |
| Products | 100.0       | 4.3            | 5.3  | 20.0 | 100.0                | 100.0 | 100.0 |

|                   | Reagents, lbs./ton | Mill | Pb Float | Zn Float | Total |
|-------------------|--------------------|------|----------|----------|-------|
| Frother No. 4     | 0.048              |      |          | 0.021    | 0.069 |
| Zn                | 0.031              |      |          | 0.032    | 0.063 |
| CaO               | 0.52               |      |          | 0.44     | 0.96  |
| NaCN              | 0.10               |      |          |          | 0.10  |
| CuSO <sub>4</sub> |                    | 18   | 13       | 13       | 1.0   |
| Time, min.        |                    |      | 20       | 20       | 20    |
| Temperature, °C.  |                    |      | 9.2-8.9  | 9.8-9.1  | ----- |
| pH                |                    |      |          |          |       |

## STANDARD TEST FOR COMPARISON, AVE. OF 6

|          | Percent Wt. | Percent Assays |      |      | Percent Distribution |       |       |
|----------|-------------|----------------|------|------|----------------------|-------|-------|
|          |             | Pb             | Zn   | Fe   | Pb                   | Zn    | Fe    |
| Pb Conc. | 8.6         | 40.7           | 13.9 | 16.1 | 81.3                 | 22.3  | 7.0   |
| Zn Conc. | 8.8         | 4.8            | 41.2 | 14.9 | 9.8                  | 68.3  | 6.7   |
| Tails.   | 82.6        | 0.46           | 0.61 | 20.7 | 8.9                  | 9.4   | 86.3  |
| Products | 100.0       | 4.3            | 5.3  | 19.8 | 100.0                | 100.0 | 100.0 |

  

|                   | Reagents, lbs./ton | Mill    | Pb Float | Zn Float | Total |
|-------------------|--------------------|---------|----------|----------|-------|
| Dowfroth          | 0.40               |         |          | 0.047    | 0.087 |
| Zn                | 0.029              |         |          | 0.030    | 0.059 |
| CaO               | 0.52               |         |          | 0.44     | 0.96  |
| NaCN              | 0.10               |         |          |          | 0.10  |
| CuSO <sub>4</sub> |                    |         |          | 1.0      | 1.0   |
| Time, min.        | 18                 |         | 13       | 13       |       |
| Temperature, °C.  |                    |         | 20       | 20       |       |
| pH                |                    | 9.2-8.9 | 9.8-9.1  |          |       |

No. 4 frother shows good properties in the flotation of this ore and is superior to Dow froth 250.

## EXAMPLE 5

Tests are carried out in rigidly standardized conditions using the well known promoting reagent "301" at a natural pH of 8.0 in a standard 2,000 gram Denver-Fahrenwald flotation machine.

The ore used contained 150 lbs. per ton pyrrhotite and 13 lbs. per ton of chalcopyrite and contained a rather unusually large proportion of reactive true colloid.

Standard tests using pine oil as frother have given very poor results.

It is thought that the invention and its advantages will be understood from the foregoing description and it is apparent that various changes may be made in the form, composition and arrangement of the ingredients without departing from the spirit and scope of the invention or sacrificing its material advantages, the forms hereinbefore described being merely preferred embodiments thereof.

What is claimed is:

1. A method for concentrating minerals by flotation comprising adding to the mineral pulp a small quantity of a polyalkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

2. A method for concentrating minerals by flotation comprising adding to the mineral pulp a small quantity of a dialkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

3. A method for concentrating minerals by flotation comprising adding to the mineral pulp a small quantity of a trialkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

4. A method for concentrating minerals by flotation comprising adding to the mineral pulp a small quantity of a trialkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

TABLE II  
[Standardised, strictly comparative, flotation tests in a 2,000-gram Denver-Fahrenwald machine, on a gold, chalcopyrite, pyrrhotite ore assaying approximately 16.8 dwts. Acc. Grind 45 minutes with 4 grams lime and 0.30 grams copper sulphate. 0.10 gram sodium-sec. butyl xanthate and the Frother as stated, at start. 2 minutes froths designated as "First Cons." Then 0.25 gram of the same xanthate, and the frother as stated. 5 minutes froths designated as "Second Cons." Residual pulp washed out of machine, designated as "Tailings."]

| Test No. | Products, Percent Weight |           |          | Assays of Products |           |                    | Units of Sulphur (percent $\times$ assay) |           |           |          | Percentage of Total Cal. Sulphur |           |           |          |
|----------|--------------------------|-----------|----------|--------------------|-----------|--------------------|-------------------------------------------|-----------|-----------|----------|----------------------------------|-----------|-----------|----------|
|          | 1st Cons.                | 2nd Cons. | Tailings | Percent Sulphur    |           | Dwt. Gold Tailings | Tailings                                  | 1st Cons. | 2nd Cons. | Tailings | Ore                              | 1st Cons. | 2nd Cons. | Tailings |
|          |                          |           |          | 1st Cons.          | 2nd Cons. |                    |                                           |           |           |          |                                  |           |           |          |
| PXX 5.   | 6.15                     | 6.05      | 87.80    | 30.48              | 23.07     | 1.15               | 4.85                                      | 187.5     | 139.6     | 101.0    | 428.1                            | 43.8      | 32.6      | 23.6     |
| PXX 7.   | 6.17                     | 6.02      | 87.81    | 29.93              | 22.52     | 0.89               | 4.85                                      | 180.2     | 135.6     | 78.3     | 304.1                            | 45.7      | 34.4      | 19.9     |
| PXX 8.   | 6.62                     | 6.61      | 86.77    | 29.24              | 20.60     | 0.65               | 4.85                                      | 193.3     | 136.2     | 56.6     | 386.1                            | 50.1      | 35.2      | 14.7     |

TABLE III

| Test No. | Substance used as Frother (in Table II) | Quantity of Substance added |           |          | Remarks                                                                                                                                                                                                                                                                                                                                                                                                        |  |  |
|----------|-----------------------------------------|-----------------------------|-----------|----------|----------------------------------------------------------------------------------------------------------------------------------------------------------------------------------------------------------------------------------------------------------------------------------------------------------------------------------------------------------------------------------------------------------------|--|--|
|          |                                         | 1st Con.                    | 2nd Con.  | Total    |                                                                                                                                                                                                                                                                                                                                                                                                                |  |  |
| PXX 5.   | 1:2:3:5 Tetramethoxybenzene             | Grams .05                   | Grams .10 | Grams 15 | Bottle warmed, added as liquid drops. Disperses rather slowly, like Pine Oil. Strong deep active, froths, not watery. Crystals dissolved in absolute alcohol for ease of measuring. (Weight (1) to 1 volume.) Very good active froths. Persistent. Crystals dissolved in alcohol, 19% w/v. Clearly much weaker than previous test PXX.7. But froths of an exceptionally good type: strong, active, persistent. |  |  |
| PXX 7.   | 1:2:3 Trimethoxybenzene                 | .046                        | .068      | .114     |                                                                                                                                                                                                                                                                                                                                                                                                                |  |  |
| PXX 8.   | 1:3:5 Trimethoxybenzene                 | .070                        | .180      | .250     |                                                                                                                                                                                                                                                                                                                                                                                                                |  |  |

TABLE IV  
[Standard Flotation Tests on a Chalcopyrite-Pyrrhotite Ore in a 2,000 gram Lab. machine.]

| Substance used as Frother                                        | Product, Percent Weight of Ore                                                         | Mineral Grade of Products          |                                      |                                        | Lbs. Mineral Per Ton Ore           |                                       | Froth Type            |
|------------------------------------------------------------------|----------------------------------------------------------------------------------------|------------------------------------|--------------------------------------|----------------------------------------|------------------------------------|---------------------------------------|-----------------------|
|                                                                  |                                                                                        | Chalco-pyrite                      | Pyrrho-tite                          | Gangue                                 | Chal.                              | Pyrr.                                 |                       |
| X.4 1, 2, 3 Tri-Methoxybenzene (0.068 g. diss. in abs. alcohol). | 1st Conc. 3.80<br>2nd Conc. 4.41<br>Comb. Conc. 8.21<br>Residue 91.79<br>Calc. Ore 100 | 13.5<br>0.8<br>6.6<br>0.06<br>0.60 | 48.2<br>66.1<br>57.8<br>2.17<br>6.74 | 38.3<br>33.2<br>35.6<br>-----<br>----- | 10.3<br>0.7<br>11.0<br>1.1<br>12.1 | 36.7<br>58.3<br>95.0<br>39.8<br>134.8 | Very good—persistent. |

poxy, isopropoxy, methoxy-ethoxy and ethoxy-ethoxy and thereafter subjecting the resulting mixture to a flotation operation.

4. A method for concentrating minerals by flotation comprising adding to the mineral pulp a small quantity of a tetraalkoxy substituted benzene as a frother, the alkoxy groups being connected to the benzene nucleus by a C—O—C ether linkage and alkoxy being selected from the group consisting of methoxy, ethoxy, normal propoxy, isopropoxy, methoxy-ethoxy and ethoxy-ethoxy and thereafter subjecting the resulting mixture to a flotation operation.

5. A process as in claim 2 wherein the frother is diethoxy benzene.

5 10

6. A process as in claim 3 wherein the frother is triethoxy benzene.

7. A process as in claim 4 wherein the frother is tetraethoxy benzene.

8. A process as in claim 1 wherein the frother is a mixture of different polyalkoxy benzenes.

References Cited in the file of this patent

UNITED STATES PATENTS

|           |               |       |               |
|-----------|---------------|-------|---------------|
| 1,902,070 | Halbig        | ----- | Mar. 21, 1933 |
| 2,561,251 | Van Aardt     | ----- | July 17, 1951 |
| 2,591,289 | Powell et al. | ----- | Apr. 1, 1952  |